

# UNITED STATES PATENT OFFICE.

PAUL F. BOVARD, OF WINONA, MINNESOTA.

## PROCESS FOR WATERPROOFING FIBROUS MATERIAL.

1,280,954.

Specification of Letters Patent. Patented Oct. 8, 1918.

No Drawing.

Application filed June 4, 1917. Serial No. 172,679.

*To all whom it may concern:*

Be it known that I, PAUL F. BOVARD, a citizen of the United States, residing at Winona, in the county of Winona and State 5 of Minnesota, have invented a new and useful Process for Waterproofing Fibrous Material, of which the following is a specification.

Its object is to render fibrous material per- 10 manently impervious to moisture, and it is particularly adapted to the treatment of animal and vegetable fibers; though it may also be applied with beneficial results to the waterproofing of mineral fibers, such as asbestos and mineral wool.

When treated as hereinafter described, the individual fibers are immune from absorption of water, and when the fibers are matted or felted together after such treatment, the 20 air cells or interstices between them are rendered less susceptible to absorption of water by reason of decrease capillary attraction of the material so treated.

The usual methods now practised are de- 25 pendent upon the adhesion of oil bases to the surfaces of the fiber; the bond depending upon the capillary attraction between the treated fiber and the oil, but water, especially if warm, breaks down this adhesion, 30 because water appears to have a greater affinity for the fibrous material than the oil.

My process consists in subjecting the fibers as hereinafter pointed out to the action of a solution of saponified oil and then fixing 35 the fatty anhydrous salt of aluminum in the fiber cells and upon the fiber surfaces.

To this end, I first provide a solution of saponified linseed oil or linseed oil soap, neutral or slightly alkaline—too much al- 40kalinity being detrimental in that it cuts the length of animal or vegetable fibers. I prefer to use a solution of linseed oil soap of from 1° Baumé to 3° Baumé at a tempera- 45ture of about 150° Fahrenheit. It is beneficial to add casein to this soap solution as a size and hardener for the water repellent precipitates, the alkalinity of the soap being sufficient to render the caesin soluble. One pound casein to 100 pounds of soap is suffi-

cient for satisfactory results. More casein 50 may be used, but this is not essential.

In this solution I immerse the fibers in a loose condition, the length of immersion depending upon the density of the fiber mass. With 1 pound dry, loose fiber to 1 gallon 55 of solution, about 30 minutes are required if the temperature is maintained at 150° Fahrenheit. The fibers should, of course, be entirely immersed during the period of the bath to insure investment.

After this treatment, the fiber is squeezed 60 thoroughly to remove the excess of soap and size and then immersed in a solution of aluminum acetate of a strength of from 1° Baumé to 4° Baumé, dependent upon the 65 class of fiber being treated. Vegetable fibers in unfelted condition are thoroughly reacted upon with a 2° Baumé solution when treating 1 pound of dry fiber to each gallon of the solution for 15 minutes.

I have specified the use of aluminum acetate, because I have found that this compound of aluminum is best fitted for my use, but it is also true that aluminum sulfate may be substituted therefor; though with 75 coarse fibers, such as are used for insulating purposes, the result is less efficient. However, I regard the use of either of these compounds of aluminum in my process as within the spirit of my invention.

The aluminum sulfate or aluminum acetate has a hardening effect upon the aluminum linoleate formed in the cells of the vegetable and animal fiber, and the presence 80 of casein adds to the permanence of the in- 85 vestment.

The excess of aluminum acetate should be squeezed from the fiber.

On thorough drying, the fibers will not take up water by capillary attraction. It 90 is necessary that all moisture be expelled in drying for satisfactory results.

Having described my invention, what I claim as new and desire to protect by Letters Patent is:

1. The method of treating fibrous material by immersing the same in a solution of saponified linseed oil and casein, then re-

60

65

70

75

80

85

95

moving the excessive moisture and again immersing the fibers in a solution of aluminum acetate, and finally drying the fibers.

2. The method of waterproofing fibrous material which consists (1) in immersing the same in a solution of saponified linseed oil and casein until the fibers are thoroughly saturated therewith, (2) in removing the

fibers from such solution and eliminating the free moisture by squeezing, (3) in immersing the fibers in a solution of an aluminum compound as specified, and finally in drying the fibers. 10

Whereof, I have hereunto subscribed my name to this specification.

PAUL F. BOVARD.